

## UNITED STATES PATENT OFFICE.

SAMUEL PEACOCK, OF WHEELING, WEST VIRGINIA.

## PROCESS OF MAKING IRON AND STEEL DIRECT.

No Drawing.

Application filed December 6, 1922. Serial No. 605,286.

*To all whom it may concern:*

Be it known that I, SAMUEL PEACOCK, a citizen of the United States, residing at Wheeling, in the county of Ohio and State of West Virginia, have invented certain new and useful Improvements in Processes of Making Iron and Steel Direct; and I do hereby declare the following to be a full, clear, and exact description of the invention, such as will enable others skilled in the art to which it appertains to make and use the same.

This is a process for making low carbon iron or steel directly from the ore in a blast furnace, and producing as a by-product a slag having the composition and properties of commercial glass.

In order that the exact process may be the better understood it is said: The modern iron-making blast furnace is a counter-current heating apparatus, in which iron oxides are reduced by carbon monoxide gas and solid carbon, and the non-ferrous components of the ore, fluxes and fuel ash are combined as fusible slags. It is essential that both the metallic iron and the slags thus produced take and hold a free running molten form; that they may be separated from each other in the hearth, and be readily withdrawn from the furnace inclosure as mobile liquids. Pure iron melts at about 2800° F., and for the necessary molten fluidity, it must be heated to about 3000° F.,—a temperature not directly obtainable by burning carbon with air. The thermo-chemical balance involved in iron formation by reducing iron oxide with carbon monoxide is strongly exothermic, and when such reduction takes place when the ore and carbon monoxide gas has been previously heated from 1000° to 1200° F., the heat liberated by the reaction is sufficient to melt the metal, notwithstanding that at the instant of its formation it exists as pure metallic iron. The molten iron thus formed, in dripping through the fuel to the hearth contacts more or less with fuel ash, white hot coke, and the hot combustion gases, and is partly reoxidized to iron oxide by carbon monoxide, and takes up carbon, silicon,

etc., and produces as an ultimate end-product a crude iron-carbon compound having a melting point about 2400° F. and a high liquid mobility at about 2500° F. This product, known commercially as cast iron, 55 has a number of uses, but its most important industrial application is in the manufacture of steel, for which purpose it is treated almost exclusively to remove wholly or in part the impurities unavoidably added to 60 the iron in the blast furnace.

Unfortunately, the steel making methods largely Bessemer or open hearth treatments are high temperature reactions in which air is used to oxidize silicon, carbon, 65 etc., and unavoidably nitrogen, carbon monoxide, metalloids oxycarbides, iron oxides and oxycarbides, hydrogen, nitrogen, dissociation products, etc., are more or less introduced into the metal. As a result for 70 steels of standard characteristics, the metal must be further treated, usually in an electric furnace, to remove the ill effects of the first refining steps. Open hearth steel making also employs iron oxides which are commonly not wholly reduced, and dissolve in 75 the steel and contribute additional undesirable impurities.

If it were possible to disregard sulphur and phosphorus a blast furnace charge could be proportioned for a slag composition of low free running temperature, and the iron thus made would be low in silicon and carbon, but by using an excess of fuel and slag, the iron would still be sufficiently impure to maintain a tapping mobility in the furnace crucible or hearth. The sulphur problem, however, precludes such operation. The sulphur goes into the furnace almost wholly as iron sulphide. The usual furnace 80 practice for sulphur removal is to proportion the fluxes to make a highly basic or calcium slag, on the assumption that a molten basic silicate in contact with iron sulphide will effect a change and produce free 85 iron and calcium sulphide. Such reaction, however, cannot range beyond the equilibrium balance, which is small; hence to remove any substantial quantity of sulphur, a 90 large proportion of such basic slag must be 95 100

used, entailing increased fuel costs and a lessened metal output per unit of plant investment. Also, the temperature must be forced to the highest obtainable in a blast 5 furnace in order to maintain a working fluidity, as a basic or "limey" slag to run freely must be heated to about 3000° F.

Further, in iron making, it is economically important to reduce the iron oxides in 10 the upper part of the furnace, by means of the carbon monoxide gases made at the tuyer zone. Carbon monoxide reduces iron oxide freely at 1000° F. But if a basic or limey slag must be used in order to eliminate sulphur, the temperature at the top of the bosh 15 should exceed 2600° F., and at this temperature the free iron made above the bosh attacks the carbon monoxide present, thus producing iron oxide and free carbon in accordance with the following equation:



That is, elemental iron is converted back to iron oxide, and such iron oxide on the 25 furnace hearth reacts with white hot coke to form iron carbide. It is at this phase that the iron silicides are formed.

It is true that these conditions are desirable in making certain grades of cast 30 iron, but for steel making it is obvious that energy is being expended to no useful end.

Again, phosphorus is present in iron ores, fluxes, etc., in the form of iron, calcium, and aluminum phosphates. These phosphates have a comparatively low melting 35 point and when fused prior to contact with red hot carbon, are reduced to phosphides. Iron phosphide dissolves in molten iron, but aluminum and calcium phosphides do 40 not. These latter phosphides react with the iron oxides present to form iron phosphides, but do not react in contact with molten iron only. At the high temperatures used in modern blast furnaces, iron oxides are 45 always present, from the top of the bosh to the tuyer zone, due to the high temperature reaction reversions; hence nearly all of the phosphorus in the furnace burden ultimately on the hearth as iron phosphide, and dissolves in the molten iron. The silicon and 50 carbon forced into the iron is a somewhat simpler reaction, due to the conditions imposed by sulphur elimination, by a very high hearth temperature, and by a very hot slag.

It will thus be seen from the foregoing that the problem of making iron or steel directly from iron oxides is beset with a great number of difficulties. To obviate 55 these difficulties it has been heretofore proposed to proceed as follows:

A blast furnace charge containing an alkali chloride has been proposed to produce a free running basic slag at a temperature of, say, 2000° F. It was thought that the

serious practical disadvantages of a very hot furnace would thus be eliminated. Now, theoretically, an alkali chloride, for example, sodium chloride in contact with fused iron sulphide and ferric oxide and in 70 an atmosphere containing not below 6% to 8% carbon monoxide, will react to form sulphur carbonyl and iron and sodium oxides, at comparatively low temperatures, but not appreciably below 2400° F. The 75 reactions may be approximated as follows:



The elimination of phosphorus as phosphorus chloride by interaction of a metal chloride and phosphate at about 2400° F. is, of course, a well known reaction, and has been the subject of repeated patent 85 applications.

But unfortunately in practice the intensely reducing atmosphere of an iron making blast furnace quickly converts the phosphates present in the furnace charge to 90 phosphides. Therefore, in the presence of sodium chloride, sodium phosphides will largely predominate by double decomposition, thus



Further, in the presence of carbon monoxide and ferric oxide, the formation of gaseous phosphorus carbonyl takes place. The specific reaction is not known to me 100 at this time, but at the temperature of the charge, approximately 2400° F., the following equation illustrates the decomposition:



The identity of the phosphorus carbonyl has not been established. But it is a gas at ordinary temperatures, and in contact with air at very low temperatures, it ignites 110 and burns with a non luminous flame, with the formation of dense clouds of phosphorus pentoxide.

I am further aware that it has been heretofore proposed to decompose iron, sulphur, 115 and phosphorus compounds in the charge by means of a dissociated metal chloride, see for, example, U. S. Patent #1061950, Simpson, et al., May 13, 1913. However, this patented process specifically denies the use 120 of carbon or carbon compounds in any of the reactions involved, except for the carburizing of previously made pure iron, the specific proportions being designated. The patented process also requires a temperature 125 of 3000° F. and upward, a degree of heat not practically obtainable in a blast furnace. The patent specifically states that "ordinary air blast furnaces of all descriptions are unsuitable for this process." 130

Thus it appears, in so far as my knowledge goes, none of the prior procedures adapted for making steel direct from the ore, have been able to get rid of 5 the sulphur present in the iron, without carrying the temperature up to, say, 3000° F. which is not only objectionable as being very difficult and costly to maintain in a blast furnace, but is also objectionable when 10 a very basic lime slag is used, because of the formation of the above mentioned iron carbides and iron silicides.

This invention, on the other hand, differs from the foregoing procedures and solves 15 the difficulties involved by the following steps: That is, in carrying out my invention, the reduction of iron oxides to metallic iron in a blast furnace is effected by the usual charges with additions containing 20 sodium chloride, or other suitable chlorides of the metals or alkali earth metals, and only sufficient lime to make a very fluid slag, at say 2400° F. and in the usual manner of operating such furnaces.

25 But the process is carried out at a somewhat lower temperature than is habitually employed in a hot blast coke furnace. More particularly stated, my process consists in the discovery that in a reducing atmosphere, 30 the sulphur and phosphorus compounds of iron that are in contact with carbon monoxide and a metal chloride such as NaCl effect such reactions that the sulphur and phosphorus present take on gaseous forms 35 at temperatures of from 2300° F. to 2400° F., and escape with the combustion gases, thus rendering it unnecessary to employ a high calcium slag at say 3000° F. to rob the iron sulphide present of its sulphur, as has 40 been the custom heretofore. And further, that because of such gaseous elimination of sulphur and phosphorus without employing extremes of temperature, (such as 3000° F.) a low carbon and silicon iron or practically a steel, is made directly from the ore, 45 in a blast furnace, employing carbon and carbon monoxide as the reducing reagents.

The charge is so proportioned that the slag formed by my process not being excessively 50 basic, is therefore very fluid and will contain little or no iron silicates; hence, this 55 slag constitutes a by-product which is suitable for direct use in making glass. The quantity of alkali metal chloride or other suitable alkali metal compound employed 60 will depend upon the quantity of the alkali metal silicate it is desired to produce and will be readily calculated by the furnace operator in each instance. Said chloride 65 suffers more or less colatilization in the process, but as its boiling point is well above 1800° F., the alkali vapor condenses on the cold burden above the bosh and is returned to the process, ultimating as a silicate and forming part of the slag. As this slag con-

tains neither sulphur, phosphorus, nor iron, it is directly available for making commercial glass, thus reimbursing all flux costs.

The ferrous metal will contain from .01% to .04% carbon, with traces only of silicon, 70 sulphur, or phosphorus. On account of the low operating temperature and low slag burden, the blast pressures are low, and both the slag and the iron may be discharged from the furnace in constant 75 streams, substantially as practiced in copper smelting, the furnace hearth constituting a forehearth effect.

Industrially the process should reduce 80 the slag and fuel burden by as much as, say, 35% to 40%, and produce a by-product in the glass making slag, which should have a commercial value, at least in excess of all flux costs. Also, as steel is produced directly by this process, the usual Bessemerizing 85 or open hearth treatment may be eliminated.

It is obvious that any metal chloride or alkali earth metal chloride whose boiling point is too high to permit the chloride to 90 escape with the combustion gases, or which is higher than say 500° C. may be employed in this process; but I prefer the use of sodium chloride or potassium chloride on account of their glass making properties. 95 By the terms metal chloride used in the claims I mean to include all chlorides of metals whose boiling points are higher than 500° C. and by the term alkali metal chlorides I mean to include the chlorides of 100 alkali earth metals.

What is claimed is:—

1. The process of making steel direct from the ore, which consists in charging a blast furnace with the usual steel making materials containing a sufficient quantity of lime and an alkali metal chloride to make a free running slag at 2400° F.; smelting the charge thus produced in the usual manner at temperatures below 2700° F. to pass off 110 the sulphur present in a gaseous form; and recovering the metal and slag produced.

2. The process of making steel direct from the ore which consists in charging a blast furnace with iron ore carbon and fluxing 115 materials containing a quantity of lime only sufficient to make a fluid slag at 2400° F. and a quantity of sodium chloride sufficient to render said slag suitable for glass making purposes; igniting said charge; maintaining the temperature below 2700° F.; and recovering the steel and slag thus produced.

3. The process of making steel direct from the ore, which consists in providing a blast furnace charge containing a quantity of lime 125 insufficient to extract the sulphur from the iron sulphide present and a quantity of sodium chloride sufficient to render the slag suitable for glass making purposes; igniting said charge; maintaining the tempera- 130

ture sufficiently high to make the desired steel and glass making slag; and recovering the latter.

4. The process of making steel direct from the ore, which consists in providing a blast furnace charge containing a quantity of lime insufficient to extract the sulphur from the iron sulphide present and a quantity of

alkali metal chloride sufficient to render the slag suitable for glass making purposes; 10 igniting said charge; maintaining the temperature sufficiently high to make the desired steel and glass making slag; and recovering the latter.

In testimony whereof I affix my signature.

SAMUEL PEACOCK.